

C. W. HAWTHORNE.  
PROCESS OF HANDLING AND ROLLING BILLETS.  
APPLICATION FILED JUNE 27, 1917.  
**1,292,462.** Patented Jan. 28, 1919.  
2 SHEETS—SHEET 1.



*Fig. 1.*



*Fig. 4.*



*Fig. 5.*



*Fig. 6.*



*Fig. 7.*

Inventor  
Charles W. Hawthorne  
By Fowler & Kennedy  
Attorneys

C. W. HAWTHORNE.

PROCESS OF HANDLING AND ROLLING BILLETS.

APPLICATION FILED JUNE 27, 1917.

1,292,462.

Patented Jan. 28, 1919.

2 SHEETS—SHEET 2.



Inventor  
Charles W. Hawthorne  
By  
Fowler & Kennedy  
Attorneys

# UNITED STATES PATENT OFFICE.

CHARLES W. HAWTHORNE, OF BUFFALO, NEW YORK, ASSIGNOR TO MORGAN CONSTRUCTION COMPANY, OF WORCESTER, MASSACHUSETTS, A CORPORATION OF MASSACHUSETTS.

## PROCESS OF HANDLING AND ROLLING BILLETS.

1,292,462.

Specification of Letters Patent. Patented Jan. 28, 1919.

Continuation of application No. 49,947, filed September 10, 1915. This application filed June 27, 1917. Serial No. 177,359.

*To all whom it may concern:*

Be it known that I, CHARLES W. HAWTHORNE, a citizen of the United States, residing at Buffalo, county of Erie, and State 5 of New York, have invented a new and useful Improvement in Processes of Handling and Rolling Billets, of which the following is a specification, accompanied by drawings forming a part of the same.

10 This invention relates to a process for handling and rolling hot billets in rolling mills, and it has for its objects to provide for rapid, easy, and certain handling and rolling of the billets without interference 15 from the scale which forms upon the billets during their heating in the furnace, and to provide means for passing the billets into the rolls without interference from or difficulty with scale or oxid formed on the surface of the billet. These and other objects 20 of invention will be set forth hereinafter in part and in part will be obvious herefrom.

This application is a continuation of the application filed by me for the same invention on the 10th day of September, 1915, Serial 25 No. 49,947, which original application Serial No. 49,947, was a division of my application filed May 15, 1915, Serial No. 28,317. The mechanism herein described by 30 which my process is carried into effect, forms no part of my present invention, it having been described in my copending application filed June 27, 1917, Serial No. 177,360.

The accompanying drawings illustrate one 35 manner of carrying out my improved process in connection with one well known type of heating furnace. In the accompanying drawings,

Figure 1 is a longitudinal sectional view 40 of the furnace in which the billets are heated.

Fig. 2 is a plan view of the delivering end of the furnace shown in sectional view, and in connection with an apparatus for delivering the billets one by one by an endwise 45 movement from the furnace, said apparatus being shown in plan view.

Fig. 3 is a transverse sectional view of the furnace at the delivery end, with the apparatus for removing the billets from the furnace shown in side elevation.

Fig. 4 is a transverse sectional view of the supporting trough 16 for the pusher rod on the plane of the broken line 4-4, Fig. 2, the pusher rod 20 being shown as lying flat upon 50 the bottom of the trough.

Fig. 5 is a transverse sectional view of the trough 16 on the plane of the broken line 5-5, Fig. 2, the pusher rod 10 being shown as having been turned one eighth of a revolution on its longitudinal axis. 60

Fig. 6 is a plan view of a water cooled inclined plate forming a part of the hearth of the furnace.

Fig. 7 is a front view of a pair of rolls representing the position of the billet in 65 one of the roll passes.

Similar reference characters refer to similar parts in the different figures.

In heating billets preparatory to rolling, according to my invention, the billets are 70 placed in the furnace side by side and closely contiguous to one another. The billets are fed along the furnace and toward the delivery end thereof whence they are removed one by one by a longitudinal movement 75 through an opening in the side wall of the furnace, and presented to the rolls of the mill. In the type of furnace shown in the accompanying drawings, the billets are pushed by a step-by-step movement toward 80 the delivery end of the furnace and along a hearth to a position opposite a delivery opening in the side wall of the furnace, through which they are pushed by suitable mechanism and presented to the rolls of the 85 rolling mill. In the above described type of furnace the tops of the billets are presented to the direct action of the heating medium, the heat and the oxygen present causing a heavy coating of oxid or scale to 90 be formed upon the tops of the billets.

In other well known types of heating furnaces, the billets are pushed by a step-by-step movement along a longitudinal track consisting of water cooled pipes, raised above 95 the bottom of the furnace, by which the heating medium is admitted to both the upper and under sides of the billets. In furnaces of this type the heavy oxid or scale will be formed upon both the upper 100 and under sides of the billets, while the sides of the billets which are in contact will be protected from the direct action of the heating medium, and will remain comparatively clean and devoid of scale. 105

In feeding the billets into the roll passes by the usually practised methods difficulty has been experienced by reason of the rolls failing to immediately grip the billets, causing a slipping of the rolls on the coating of 110

oxid or scale on the top or bottom of the billets. The scale also, after the rolls have caught the billet, is broken and rolled into the metal, more or less impairing its quality and texture. In order to obviate the injurious effect of the scale upon the surface of the rolls, it has been found necessary to harden the surface of the rolls, thereby making it difficult to redress the surface of the rolls in order to preserve the desired contour and size of the roll passes. The usually practised method is therefore subject to various serious objections, especially when it is desired to roll the metal to exact dimensions. By my improved process I maintain the two parallel and vertical sides upon each billet, comparatively free from oxid or scale and confining the scale formed on the billets to one or both of the remaining sides. When the billet has been sufficiently heated and has been brought into position to be delivered through an opening in the side wall of the furnace, I push the billet by an endwise movement into the grip of the rolls of the mill by a mechanism which produces a positive rotative movement of the billet in order to bring its contacting or scale-free sides into contact with the upper and lower surfaces of the roll passes, to insure that the scale free sides of the billet, or the sides which were in contact during its passage through the furnace, shall contact only with the surfaces of the rolls, by which the reduction or compression of the metal is effected. By this means I not only obviate the various disadvantages incident to the rolling of billets by the usually practised methods, but I also substantially free the rolled metal or finished product from the injurious effects due to crowding the scale into the mass of rolled metal. This result I accomplish by bringing the sides of the billets having a heavy scale thereon into vertical positions at right angles to the axes of the rolls, so that when the billet becomes compressed by the action of the rolls the scale present upon the vertical sides of the billet will become buckled by its compression, and free itself from the billet.

I am also able to use rolls comparatively soft, and easily returned to preserve the size of its passes. I am aware that it is not new to feed billets in a continuous row through a heating furnace by means of a step-by-step movement, also that it is not new to feed billets from the furnace to the roll by a pushing bar. Means have also been employed for rotating billets within a heating furnace by which heat is more uniformly applied to all the sides of the billet with the consequent formation of scale.

In the above description and in the accompanying drawings, I have illustrated

the successive steps of my improved process, which so far as I am aware is broadly new in the art of rolling metal.

Referring to the accompanying drawings, which illustrate one manner of carrying my process into practice, 1 denotes a heating furnace having a longitudinal hearth 2, over which the row of billets 3 are moved by a step-by-step movement as each individual billet is entered into the furnace by 75 a reciprocating pusher 4. As the billets are moved through the furnace their vertical sides 5, Fig. 1, will be held in close contact and thereby protected from the direct action of the heating medium, while the upper 80 surfaces 6 of the billets will gradually accumulate scale or oxid, which becomes sufficiently heavy as the billets approach the delivery opening 7 to interfere with the rolling of the billet by the usually practised 85 method, in which the scaled side of the billet is brought into contact with the rolls. The accumulated scale is indicated in Fig. 1 by the heavy line 8.

In the illustrated manner of carrying my 90 process into practice, I deliver the billet to the reducing roll 9 of the mill by means of a push bar 10, to which a longitudinally reciprocating movement is given by means of a motor 11, preferably reversing, which 95 drives the pinch rolls 12 and 13 running in frictional contact with the upper and under surfaces of the bar 10 which is preferably rectangular in cross section.

The advancing end of the bar 10 is bifurcated at 14 and suitably shaped to engage the end of the billet. The bar 10 is given a quarter twist, as at 15, Fig. 2. As the twisted section 15 passes between the rolls 12 and 13 a quarter twist will be imparted 105 to the bar 10 and to the billet engaged thereby, causing the billet to be turned exactly one quarter way around, and to present the sides 5, which are free from scale, to the contact of the rolls, and bringing the scale 110 coated side 6 at right angles to the axes of the rolls, causing the scale to be loosened and removed by the compression of the billet.

The bar 10, in the present instance, is supported at the rear of the rolls 12 and 13 by a trough 16 capable of swinging on a pivot 17, and hung at its rear end by a flexible connection with an elevated support, to allow a lateral motion to be imparted to 120 the advancing end of the bar. In order to cool the end of the bar 10 entering the furnace, a sprinkler 18 is employed, supplied by a swinging pipe 19. If desired, a water cooled plate 20 may be placed in the hearth 125 to assist in guiding the bar 10. In carrying my process into practice the bar 10 is pushed forward by the rotation of the rolls 12 and 13, and allowed to swing on the pivot 17 by means of a handle 21.

I claim,

1. The herein described process of handling and rolling billets, consisting in pushing the billets in a continuous row from the receiving to the delivery end of a heating chamber, with the parallel and vertical sides of the billets in contact, feeding a billet from the row by an endwise movement from the heating chamber to a pair of rolls, and 10 positively imparting a quarter turn to each billet during said endwise movement.

2. The herein described process of handling and rolling billets, consisting in heating the billets to a rolling heat in a suitable 15 heating chamber, protecting two opposite sides of the billet from the direct action of the heating medium, feeding the heated billet from the heating chamber to a pair of rolls, and bringing the protected and par-

allel sides of the billet into a position parallel with the axes of said rolls during said feeding movement of the billet.

3. The herein described process of handling and rolling billets, consisting in passing the billets through a heating chamber, 25 with their contiguous sides in contact to reduce the formation of scale thereon, delivering said billets by an endwise movement to a stand of rolls and positively turning the billets a predetermined amount during their endwise movement to present the relatively unscaled surfaces to the compressing surfaces of said rolls.

Dated this twenty third day of June, 1917.

CHARLES W. HAWTHORNE.

Witnesses:

KARL O. McCUSAULAND,  
W. G. MOWAT.